

Patented Aug. 27, 1935

2,012,553

## UNITED STATES PATENT OFFICE

2,012,553

DYING OF CELLULOSE ESTERS AND  
ETHERS

Erwin Thoma, Frankfort-on-the-Main-Hochst,  
Germany, assignor to General Aniline Works,  
Inc., New York, N. Y., a corporation of Dela-  
ware

No Drawing. Application November 29, 1933,  
Serial No. 700,367. In Germany December 3,  
1932

6 Claims. (Cl. 8—5)

The present invention relates to the manufacture of dyeings on fibrous materials made of cellulose esters or ethers and to the dyed materials, more particularly it relates to a process which 5 comprises applying to the said fibrous materials a suitable amino compound, free from sulfonic acid groups, capable of forming a diazo component, diazotizing the amino compound on the fiber and developing (coupling) with a 5-keto-4.5-di-10 hydropyrazole compound of the general formula:



wherein  $\text{R}_1$  stands for a radical of the benzene series and  $\text{R}_2$  for  $\text{COOH}$ ,  $\text{CONH}_2$ ,  $\text{CONH-aryl}$ , or 20 for an esterified carboxylic acid group.

The technical advance attained according to the present invention resides in the fact that the dyeings produced on fibrous materials made of cellulose esters or ethers by means of the above defined group of 5-keto-4.5-dihydropyrazole compounds possess good fastness properties and can be well discharged, yielding excellent white discharge effects when treated with reducing discharging agents in known manner. Developing 30 components of such properties are highly desired in the art of dyeing cellulose esters and ethers by means of the class of the so-called developing dyes.

The dyeings obtainable, for instance, by coupling on the fiber a diazotized amino compound with 1-phenyl-3-methyl-5-pyrazolone cannot be discharged or can only insufficiently be discharged by means of reducing discharging agents. The

dyeings obtainable from 1-nitroaryl-3-methyl-5-pyrazolones, for instance, from 1-meta- or 1-para-nitrophenyl-3-methyl-5-pyrazolone, according to German Patent No. 284,695, also cannot be sufficiently discharged.

The production of the dyeings may be carried out in the usual manner. For instance, a dye-bath is prepared by dissolving about 1% of the amino compound, calculated on the weight of the goods, in water while adding a sufficient quantity of hydrochloric acid or formic acid to obtain a solution. In this solution acetate silk or other textile material made of cellulose esters or ethers are handled while slowly raising the temperature and heating for about  $\frac{1}{2}$  to 1 hour at about 50° C. to about 75° C. To the dye-bath about 5% to 10% of sodium acetate, calculated upon the weight of the goods, are advantageously added during the dyeing operation. Thereupon, the material is diazotized on the fiber in the usual manner in a freshly prepared bath, and the dyeing is then developed for about  $\frac{1}{2}$  to about 1 hour at about 50° C. to about 75° C. in another bath having a neutral or weak acetic acid reaction and containing the necessary quantity, say 3 per cent, of the 5-keto-4.5-dihydropyrazole compound, calculated upon the weight of the goods.

The amino compound may alternatively be used in the form of a suspension or emulsion in a soap bath or in the presence of any other dispersing medium. The amino compound may then be diazotized and the dyeing be developed as above described.

In the following table a number of dyeings, obtainable according to the present invention, is disclosed. It is, however, understood that the invention is not restricted to the particular combinations shown:

|    | Diazo component                                                                              | Coupling component                                                  | Tint           |    |
|----|----------------------------------------------------------------------------------------------|---------------------------------------------------------------------|----------------|----|
| 40 |                                                                                              |                                                                     |                | 40 |
| 1  | $\text{H}_2\text{N}-\text{C}_6\text{H}_4-\text{N}=\text{N}-\text{C}_6\text{H}_4-\text{NH}_2$ | 1-phenyl-5-keto-4.5-dihydropyrazole-3-carboxylic acid methyl ester. | Orange-yellow. |    |
| 45 | Do.....                                                                                      | 1-phenyl-5-keto-4.5-dihydropyrazole-3-carboxylic acid amide.        | Orange-red.    | 45 |
| 2  | Do.....                                                                                      | 3-methyl-5-keto-4.5-dihydropyrazole.....                            | Gold-yellow.   |    |
| 3  | Do.....                                                                                      | 5-keto-4.5-dihydropyrazole-3-carboxylic acid.....                   | Orange.        |    |
| 4  | Do.....                                                                                      | 5-keto-4.5-dihydropyrazole-3-carboxylic acid-ethyl ester.           | Do.            |    |
| 5  | Do.....                                                                                      | 1,3-dimethyl-5-keto-4.5-dihydropyrazole.....                        | Gold-yellow.   | 50 |
| 6  | Do.....                                                                                      | 3-phenyl-5-keto-4.5-dihydropyrazole.....                            | Orange.        |    |
| 7  | Do.....                                                                                      | 5-keto-4.5-dihydropyrazole.....                                     | Yellow.        |    |
| 8  | Do.....                                                                                      | 5-keto-4.5-dihydropyrazole-3-carboxylic acid amide.....             | Orange-red.    | 55 |
| 9  | Do.....                                                                                      | 3-phenyl-5-keto-4.5-dihydropyrazole-1-carboxylic acid ethyl ester.  | Gold-yellow.   |    |
| 10 | Do.....                                                                                      | 3-methyl-5-keto-4.5-dihydropyrazole-1-carboxylic acid anilide.      | Do.            |    |
| 11 | $\text{H}_2\text{N}-\text{C}_6\text{H}_4-\text{N}=\text{N}-\text{C}_6\text{H}_4-\text{NH}_2$ | 1-methyl-3-phenyl-5-keto-4.5-dihydropyrazole.....                   | Orange-yellow. | 60 |
| 12 | Do.....                                                                                      |                                                                     |                |    |

|       | Diazo component   | Coupling component                                                            | Tint               |
|-------|-------------------|-------------------------------------------------------------------------------|--------------------|
| 13    |                   | 1-methyl-5-keto-4,5-dihydropyrazole                                           | Gold-yellow.       |
| 14    | Do.               | 1-methyl-5-keto-4,5-dihydropyrazole-3-carboxylic acid ethyl ester.            | Orange.            |
| 15    | Do.               | 1-methyl-5-keto-4,5-dihydropyrazole-3-carboxylic acid amide.                  | Do.                |
| 10 16 | Do.               | 1-ortho-nitrophenyl-5-keto-4,5-dihydropyrazole-3-carboxylic acid ethyl ester. | Gold-orange.       |
| 17    |                   | 3-methyl-5-keto-4,5-dihydropyrazole                                           | 10<br>Gold-yellow. |
| 15    |                   | 1-phenyl-5-keto-4,5-dihydropyrazole-3-carboxylic acid methyl ester.           | Reddish-orange. 15 |
| 18    |                   |                                                                               |                    |
| 19    | Do.               | 1-phenyl-5-keto-4,5-dihydropyrazole-3-carboxylic acid ethyl ester.            | Orange-red.        |
| 20 20 | Do.               | 1-phenyl-5-keto-4,5-dihydropyrazole-3-carboxylic acid amide.                  | Do. 20             |
| 21    | Do.               | 1-phenyl-5-keto-4,5-dihydropyrazole-3-carboxylic acid anilide.                | Scarlet.           |
| 22    | Do.               | 5-keto-4,5-dihydropyrazole-3-carboxylic acid.                                 | Red-orange.        |
| 25 23 | Do.               | 5-keto-4,5-dihydropyrazole-3-carboxylic acid ethyl ester.                     | Do. 25             |
| 24    | Do.               | 3-methyl-5-keto-4,5-dihydropyrazole-1-carboxylic acid ethyl ester.            | Gold-orange.       |
| 25    | Do.               | 3-methyl-5-keto-4,5-dihydropyrazole-1-carboxylic acid amide.                  | Orange.            |
| 30 26 | Do.               | 3-phenyl-5-keto-4,5-dihydropyrazole-1-carboxylic acid amide.                  | Do. 30             |
| 27    | Do.               | 1-phenyl-5-keto-4,5-dihydropyrazole-3-carboxylic acid...                      | Reddish-orange.    |
| 28    | Para-nitroaniline | 1-phenyl-5-keto-4,5-dihydropyrazole-3-carboxylic acid ethyl ester.            | Greenish-yellow.   |
| 35    |                   | 3-methyl-5-keto-4,5-dihydropyrazole-1-carboxylic acid anilide.                | Scarlet-red. 35    |
| 29    |                   |                                                                               |                    |
| 30    | Do.               | 1-phenyl-5-keto-4,5-dihydropyrazole-3-carboxylic acid amide.                  | Red-brown.         |
| 40 31 | Do.               | 1-phenyl-5-keto-4,5-dihydropyrazole-3-carboxylic acid methyl ester.           | 40<br>Currant.     |
| 32    | Do.               | 1,3-dimethyl-5-keto-4,5-dihydropyrazole.                                      | Red.               |
| 33    | Do.               | 3-phenyl-5-keto-4,5-dihydropyrazole.                                          | Violet-brown.      |
| 45 34 | Do.               | 5-keto-4,5-dihydropyrazole-3-carboxylic acid.                                 | Violet. 45         |
| 35    | Do.               | 1-methyl-3-phenyl-5-keto-4,5-dihydropyrazole.                                 | Bluish-red.        |
| 36    |                   | 1-phenyl-5-keto-4,5-dihydropyrazole-3-carboxylic acid ethyl ester.            | Do. 50<br>Currant. |
| 50    |                   |                                                                               |                    |
| 37    | Do.               | 3-methyl-5-keto-4,5-dihydropyrazole.                                          | Brown-red.         |
| 38    |                   | 1-methyl-5-keto-4,5-dihydropyrazole-3-carboxylic acid methyl ester.           | Gold-yellow.       |
| 55 39 | Do.               | 1-methyl-5-keto-4,5-dihydropyrazole-3-carboxylic acid.                        | Orange. 55         |
| 40    | Do.               |                                                                               | Orange-brown.      |
| 41    |                   | do.                                                                           | Do. 60             |
| 42    |                   | do.                                                                           | Brown.             |

By replacing in the above defined combinations the amino-azo-compounds, used as diazo components, by other amino-azo-compounds, for instance those which contain alkyl-, halogen-, nitro- and dialkyl-amino groups, or by diamino-azo-aryl compounds, or by diamino-aryl compounds, such as dianisidine, tolidine, etc., or by mono-amines, such as naphthyl-amine, para-

nitraniline or others, there are obtained dyeings which, in contradistinction to those which are obtainable by means of the same bases and with 70 1-phenyl-3-methyl-5-pyrazolones can well be discharged, yielding white discharge effects.

I claim:

1. A process of producing dyeings on fibrous materials of the group consisting of cellulose

esters and ethers, which dyeings can be well discharged, which comprises applying to the material an amino compound, free from sulfonic acid groups, capable of forming a diazo compound, 5 diazotizing the amino compound on the fiber and developing with a coupling component of the general formula.



15

wherein R<sub>1</sub> stands for a radical of the benzene series and R<sub>2</sub> for a substituent selected from the group consisting of COOH, CONH<sub>2</sub>, CONH-aryl 10 and an esterified carboxylic acid group.

20 2. A process of producing dyeings on fibrous materials of the group consisting of cellulose esters and ethers, which dyeings can be well discharged, which comprises applying to the material an amino-monoazo dyestuff of the benzene series, free from sulfonic acid groups, diazotizing 25 the amino compound on the fiber and devel-

oping with a coupling component of the general formula:



wherein R<sub>1</sub> stands for a radical of the benzene series and R<sub>2</sub> for a substituent selected from the group consisting of COOH, CONH<sub>2</sub>, CONH-aryl 10 and an esterified carboxylic acid group.

3. A process of producing dyeings on acetate silk, which dyeings can be well discharged, which comprises treating acetate silk in a bath containing 15 4-amino-3-methoxybenzene-azo-3'-carboxybenzene, diazotizing on the fiber and coupling with 1-phenyl-5-keto-4,5-dihydropyrazole-3-carboxylic acid ethyl ester.

4. Fibrous materials of the group consisting of cellulose esters and ethers, dyed with dyestuffs 20 according to claim 1.

5. Fibrous materials of the group consisting of cellulose esters and ethers, dyed with dyestuffs according to claim 2.

6. Acetate silk dyed with dyestuffs according 25 to claim 3.

ERWIN THOMA.